

J. S. McGEHEE.

ROOFING.

APPLICATION FILED MAY 12, 1916.

1,226,547.

Patented May 15, 1917.



WITNESSES

J. S. McGehee  
F. T. Chapman

John S. McGehee, INVENTOR

BY

E. J. Siggins

ATTORNEY

106-92

## UNITED STATES PATENT OFFICE.

JOHN SIMEON McGEHEE, OF PALMERSVILLE, TENNESSEE, ASSIGNOR OF ONE-HALF TO  
ALBERT H. BRAUN, OF PALMERSVILLE, TENNESSEE.

## ROOFING.

1,226,547.

Specification of Letters Patent. Patented May 15, 1917.

Application filed May 12, 1916. Serial No. 97,167.

*To all whom it may concern:*

Be it known that I, JOHN S. McGEHEE, a citizen of the United States, residing at Palmersville, in the county of Weakley and State of Tennessee, have invented a new and useful Roofing, of which the following is a specification.

This invention has reference to roofing, and its object is to provide a substitute for shingles and other roofing which may be applied with a trowel and which, moreover, is fire and waterproof.

The roofing while intended particularly for a roof covering, may be applied to side walls, or wherever a covering to which the roofing is adapted may be employed. However, for the sake of simplicity of description the invention will be referred to as a roofing without thereby limiting the uses of the invention to such particular purpose.

In accordance with the present invention a suitable foundation of laths or strips is provided upon supporting timbers, and such strips are covered by a fine mesh wire screen which in turn is covered by a coarse mesh wire screen, and to the wire screening there is applied a composition of materials mixed in suitable proportions, and in a condition permitting the application by means of a trowel or other suitable tool. The composition dries hard and firm, hardening slowly with freedom from cracking, and when completed is both weather and fireproof with a smooth, substantially glazed surface.

The invention will be best understood from a consideration of the following detailed description, taken in connection with the accompanying drawing forming part of this specification, with the further understanding that while the drawings show a practical form of the invention, the latter is not confined to any strict conformity with the showing of the drawings, but may be changed and modified as long as the changes and modifications come within the scope of the appended claims.

In the drawing, the figure is a perspective view to a certain extent schematically representing a small section of a roof provided with the roofing of the present invention.

In carrying out the invention, the supports to which the roofing is to be applied, which supports are not shown in the drawing, are covered with strips or laths 1 suit-

ably spaced apart, say, about half an inch, so that there is no buckling of the laths should the latter swell from any cause. Covering the laths is a layer 2 of fine mesh wire screen held to the laths by staples 3 or otherwise, and covering the screen 2 is a layer of wire screen 4 which may be of about half inch mesh, although any particular mesh is not obligatory. The screen covering 4 is held in place by staples 5 or in any other suitable way. The purpose of the screen covering 4 is to provide key seats for anchoring a layer 6, of a composition to be described, to the basic portion of the roof covering, while the fine mesh wire screen 2 prevents passage of the composition to the spaces between the laths, and so far as any of the composition 6 which may reach the wire screen 2 is concerned, the latter will act as an anchoring means therefor.

The composition covering 6 is applied in a layer of, say, half an inch in thickness, and in strips of, say, about two feet wide extending from the eaves to the ridge or comb of the roof, each strip being separated from its neighbor by a space of, say, half an inch, and such a space being indicated at 7 in the drawing.

The composition 6 is made up of sand, cement, red oxid of iron, yellow ocher, plaster of Paris, saltpeter, alum, granulated sugar and sulfur, with enough water to produce a workable plaster capable of being applied to the basic portion of the roofing with a trowel or other suitable tool.

As an example of the composition, a certain quantity is made up of one hundred pounds of good clean sand, one hundred pounds of good cement, one and one-quarter pounds of red oxid of iron, one-quarter pound of yellow ocher, one pound of builder's plaster of Paris, one ounce of saltpeter, one-half ounce of alum, one pound of granulated sugar, and one pound of sulfur.

The sand, cement, red oxid of iron, ocher, and plaster of Paris are thoroughly mixed dry. The saltpeter, alum, sugar and sulfur in the quantities given above are dissolved in one gallon of boiling water, and when cool the solution is strained and then mixed with the first-named ingredients with sufficient additional water to make a trowel mortar.

The roofing composition is applied in

strips as stated, with spaces 7 between the strips until the whole roof or space to be covered is finished, and then the various strips are kept damp until thoroughly set, 5 this being accomplished by covering the whole roof with sacking and keeping the sacking wet. Then the narrow spaces 7 are filled in with the same composition packed in with a trowel and allowed to set. Finally 10 a suitable quantity of cement is mixed with enough of the solution made up of saltpeter, alum, sugar, sulfur and water to produce a thin paste, thin enough to be applied to the applied roofing composition with a 15 brush, and this is then smoothed down with a trowel to fill all crevices and holes and to produce a finishing glaze adding to the appearance of the roof. The filling for the space 7 is indicated at 8, and the final 20 brushed-on coating is indicated at 9, the filling 8 being slightly pointed if desired to produce a suitable effect upon the roof.

The plaster of Paris added to the cement and sand makes the composition firmer than 25 when the plaster of Paris is omitted. The red oxid of iron and the yellow ocher serve as coloring matters. The saltpeter is used to keep the composition from hardening too fast and cracking, and also serves as an atmosphere feeder to cause the crystallization 30 of the ingredients. The sulfur and other of the ingredients contribute to the gloss, and all the ingredients act to produce a firm and durable roofing free from liability of crack 35 and thoroughly resistant to weather conditions.

It will be understood, of course, that the coloring matters will be varied in accord-

ance with the color it is desired the roofing should have. 40

The composition may be made up into shingles, but it is advantageous to apply it as described, for the gutters and valleys may be formed of the composition in one piece with and at the same time the roof is 45 produced.

What is claimed is:—

1. A roofing composition comprising sand, cement, plaster of Paris, saltpeter, alum, sugar and sulfur. 50

2. A roofing composition, comprising sand, cement, plaster of Paris, saltpeter, alum, sugar and sulfur in substantially the parts of one hundred pounds of sand, one hundred pounds of cement, one pound each of plaster of Paris, sugar and sulfur, one ounce of saltpeter, one-half ounce of alum, coloring matter and water. 55

3. A roofing compound consisting of sand, cement, plaster of Paris, red oxid of iron, and yellow ocher mixed dry in substantially the proportions described, a solution of saltpeter, alum, sugar and sulfur substantially in the proportions described, and water in 60 sufficient quantity to make the composition of the consistency of trowel mortar. 65

4. A compound comprising cement, saltpeter, alum, sugar, sulfur and water, in substantially the proportions described. 70

In testimony that I claim the foregoing as my own I have hereto affixed my signature in the presence of two witnesses.

JOHN SIMEON McGEHEE.

Witnesses:

A. H. BRAUN,  
C. W. PENTECOST.

Copies of this patent may be obtained for five cents each, by addressing the "Commissioner of Patents, Washington, D. C."